

Patented Feb. 15, 1927.

1,617,616

# UNITED STATES PATENT OFFICE.

EDWARD G. CAUGHEY, OF SEWICKLEY, PENNSYLVANIA, ASSIGNOR TO EDGEWATER STEEL COMPANY, OF PITTSBURGH, PENNSYLVANIA, A CORPORATION OF PENNSYLVANIA.

## PROCESS OF RENDERING IRON AND STEEL NONOXIDIZABLE AND ARTICLES PRODUCED THEREBY.

No Drawing.

Application filed January 26, 1922. Serial No. 532,025.

This invention relates in general to the protection of iron or steel from oxidation and particularly where such steel or iron is subjected to high temperatures as in annealing boxes, carbonizing cases, furnace parts, etc. Annealing boxes may be taken as an example of an excellent use of the invention. Such boxes are subjected to temperatures as high as 2000° Fahrenheit and at this and intervening temperatures steel oxidizes very rapidly, as is readily observable upon comparing the weight of an annealing box after a considerable number of uses with its initial weight, until finally the walls become so thin that they must be discarded.

Another excellent use for the invention is in pots for hardening gears and other such articles. These pots, as ordinarily constructed of cast steel, last about 630 total hours in the furnace. The gears are placed in them surrounded by carbonizing material, the pot sealed up and placed in the furnace for about 18 hours at a time. After the first such heat treatment the pot begins to scale off on the outside, due to oxidation, and to absorb carbon on the inside. After about 630 hours the walls become so thin and so impregnated with carbonizing material that they must be discarded.

My invention has for a principal object the provision of a material which will not oxidize nor absorb the carbonizing elements in which the steel to be carbonized has been packed at this high temperature and which accordingly may be used indefinitely without permanent deterioration. In connection with the carbonizing pots it may be mentioned that my material shows no scaling after the first treatment, no loss of weight after about a 1050 hour test given it. Indeed after the prolonged test given it the material could not be said to have changed color.

The invention relates also to the process of rendering iron or steel non-oxidizable at high temperatures, and also to a process for maintaining such material in the original structural condition. I have found that material embodying my invention, if left in the ordinary room or at atmospheric temperatures, gradually suffers structural deterioration and as a part of my present inven-

tion I have discovered a process for correcting such deterioration so that properly handled the material may maintain its desirable qualities indefinitely.

The process of treating the steel to form the material embodying my invention consists essentially of incorporating in it a quantity of aluminum designed to produce a resultant mixture best adapted to resist oxidation and the absorption of carbonizing and other materials at high temperatures. I dissolve an amount of aluminum in the steel, determined by the temperature at which protection against oxidation is most desired, i. e., calculated to present maximum resistance to oxidation at the highest temperature to which the material is ordinarily subjected. I have found by experiment that in the case of an annealing box to resist high temperatures and made from low carbon steel, material with approximately 12% to 15% of aluminum in the steel gives satisfactory results. The two materials are melted and united in molten condition. It is believed that the aluminum combines with the iron to form an iron aluminum compound and that after the metal has solidified this iron aluminum compound is dissolved in the remainder of the metal as a solid solvent. I have found that this material cast into annealing boxes, carbonizing pots, etc., will permanently resist oxidation at the high temperatures such articles are ordinarily subjected to. I have found, however, that this material upon being allowed to stand at atmospheric temperatures undergoes a structural change and deteriorates and my researches indicate that the steel, being saturated at higher temperatures with the aluminum compound, is super-saturated at atmospheric temperatures and gradually and slowly the aluminum compound passes out of solution collecting between the grains and along their cleavage planes, thus weakening their natural bond. This may be overcome and corrected by periodic or occasional heating of the material to a temperature not exceeding that at which the annealing boxes, carbonizing pots, or other articles are designed to withstand in service. This may be accomplished by especial heating or as an incident to the use of the article made of the material. I have discovered that the

original condition is reestablished and that the aluminum or the aluminum iron compound passes back into solution, thus restoring the original physical properties of the material.

While in the claims the expression "iron" is used it will be understood that by this term it is intended to include steel as well. It is further stated that this material is very hard and that the invention contemplates the use of a lower percentage of aluminum with resulting lower percentage of aluminum compound in solution in order to provide a material more readily forged and worked. It will also be understood that in so far as the prevention of absorption of carbon is concerned in carbonizing pots and the like where the invention is employed, my present intention is that the absorption is prevented by the saturation at the working temperature of the iron by the iron aluminum compound. In accordance with the best present advices carbon enters into iron or steel by forming an iron carbide which passes into solution in the iron above its critical point so that if the iron be saturated this action cannot occur to any appreciable extent.

It is thought that the invention and many of its attendant advantages will be understood from the foregoing description, and it will be apparent that various changes may be made without departing from the spirit and scope of the invention or sacrificing all of its material advantages, the form hereinbefore described being merely a preferred embodiment thereof.

I claim:

1. A process of rendering iron non-oxidizable or resistant to oxidation at high temperatures, which includes, incorporating in the iron as a solid solvent a quantity of aluminum to form a saturated solution in said solvent at the temperature at which it is particularly desired to prevent oxidation.

2. A process of rendering iron non-oxidizable or resistant to oxidation at high temperatures, which includes, incorporating in the iron as a solid solvent a quantity of aluminum to form a saturated solution in said solvent at the temperature at which it is particularly desired to prevent oxidation and bringing said iron to said temperature

upon occasion to redissolve any aluminum compound separated out at lower intervening temperatures.

3. A process of rendering iron non-oxidizable or resistant to oxidation at high temperatures, which includes, incorporating in the iron a quantity of aluminum in amount appropriate to cause structural deterioration over protracted periods at atmospheric temperatures and heating the iron to said high temperatures upon occasion to restore the structural quality of said iron.

4. A process of rendering iron non-oxidizable or resistant to oxidation at high temperatures, which comprises, dissolving in the iron as a solid solvent a quantity of aluminum appropriate to form a saturated solution at approximately the highest working temperature to which the treated iron is subjected in service.

5. A metal article adapted to be subjected to high temperatures in service and formed of a material non-oxidizable by such temperatures, comprising iron as a solvent in which has been dissolved a quantity of aluminum, approximately in amount appropriate to form a saturated solution of aluminum compound in the iron at the temperature at which oxidation is to be prevented.

6. A metal article adapted to be subjected to high temperatures in service and formed of a material non-oxidizable by such temperatures, comprising iron with a quantity of aluminum dissolved in the iron as a solid solvent, in amount appropriate to form a saturated solution at the highest working temperatures to which said material is to be subjected.

7. A metal article adapted to be subjected to high temperatures in service and formed of a material non-oxidizable by such temperatures, comprising a mixture of iron and aluminum in amount appropriate to prevent oxidation, the relation of said iron and said aluminum in said mixture being such that structural deterioration results from protracted interrupted subjection of the mixture to atmospheric temperature, and re-establishment of the original structure obtainable by heating of said iron to a higher temperature.

EDWARD G. CAUGHEY.